

March 27, 1928.

1,663,954

R. B. RESPRESS

BUFFING LEATHER SUBSTITUTE AND PROCESS OF MAKING THE SAME

Filed June 5, 1920

*Fig. 7*



*Fig. 1*



*Fig. 6*



*Fig. 2*



*Fig. 3*



*Fig. 4*



*Fig. 5*



Executor:  
Roland B. Respess  
by Roberts, Roberts & Culmar  
Attest.

Patented Mar. 27, 1928.

1,663,954

# UNITED STATES PATENT OFFICE.

ROLAND B. RESPESS, OF NEW YORK, N. Y., ASSIGNOR, BY MESNE ASSIGNMENTS, TO  
RESPRO INC., OF CRANSTON, RHODE ISLAND, A CORPORATION OF RHODE ISLAND.

## BUFFING-LEATHER SUBSTITUTE AND PROCESS OF MAKING THE SAME.

Application filed June 5, 1920. Serial No. 386,713.

This invention relates to a buffing leather substitute and the process for making the same and its organization is particularly directed to an improvement in the invention 5 described in my application for unwoven fabric and process for making the same, filed March 11th, 1919, Serial Number 282,018 as applied to the manufacture of very thin leather substitute. 10 It has heretofore been the practice to make leather buffing from very thin cuts from the surface of genuine leather, or from very thin splits of genuine leather coated with a surface dressing. Artificial leather buffing has 15 also been made from very thin sheeting or cheese cloth which is coated with a cellulose compound.

The purpose of my invention is to make a very thin sheet of buffing leather substitute 20 composed of untwisted and unwoven cotton fibers for the backing thereof, with a surface coating of cellulose or other leather surface dressing which will penetrate into the matted fiber backing. The product produced 25 by this process is very strong, and may therefore be used in thin sheets. The product also will have the quality of being easily cemented to card board for book binding and the like, inasmuch as the fibrous backing 30 gives a surface to which ordinary paste mixtures adhere readily.

Fig. 1 is a diagrammatic side elevation illustrating the various successive steps in the process herein described.

35 Fig. 2 is a fragmentary section substantially on the line 2—2 of Fig. 1 showing the construction of the original bat or sheet of unspun fibres.

40 Fig. 3 is a similar section on the line 3—3 of Fig. 1 showing the bat or sheet after impregnation.

45 Fig. 4 is a similar section on the line 4—4 of Fig. 1 showing the bat or sheet after drying and with a coating of adhesive applied to one side thereof;

50 Fig. 5 is a section on the line 5—5 of Fig. 1 showing a composite sheet comprising the original bat combined with a web of textile fabric.

55 Fig. 6 is a section on the line 6—6 of Fig. 1 showing the composite sheet as having been provided with a coating of surface dressing upon the exposed surface of the bat; and

Fig. 7 is a section substantially on the line

7—7 of Fig. 1 showing the finished artificial 55 buffing leather formed in accordance with the present process.

The first step in the process consists in making a bat or sheet of unwoven, unspun fibers preferably of cotton, the operation being performed by a carding or garnetting machine of usual type such as is used in the manufacture of wadding, batting or felt. For the purpose of this invention it is desirable that this bat or sheet be formed of a 60 65 plurality of distinct strata or layers superposed one on the other, so that the finished bat has a plane or planes of cleavage intermediate its outer surfaces.

The next step is to pass the sheet roll of 70 prepared batting to a saturating machine where it is impregnated with an adhesive agent, after which it is dried and pressed. In this step I prefer to pass the sheet to a conveying belt which passes between pressure rollers just after the application of the adhesive agent to the fiber sheet. The rollers press the adhesive agent into the fibrous sheet. Next the sheet passes to a drying 75 chamber where the solvent of the adhesive 80 agent is evaporated and the dried sheet is then pressed under tension.

The next step is to attach the sheet to a woven fabric. In this step the fiber sheet is 85 coated with an adhesive agent on one side of the sheet and a woven fabric sheet is similarly coated on one side or surface and the two coated surfaces superimposed on each other and subjected to pressure. I usually prefer to use a rubber compound containing 90 vulcanizing agents as the adhesive agent and when it is used the product is subjected to heat and vulcanized. It is frequently desired also to cement an untwisted fiber sheet to both sides of the woven fabric and in such 95 case the same process is used for attaching the fiber sheet to both sides of the woven sheet.

When the sheet is not to be made as a by-product to the double texture fabric as described and is used without attaching it 100 to a woven sheet, an additional step may be to subject the sheet to a curing process, to further set the adhesive agent and if a rubber compound is used as the adhesive agent the sheet may be subjected to heat and vulcanized. In some cases I may use the dried 105 and pressed sheet without any curing process.

- The next step in the process is to coat the surface of the untwisted fibrous sheet with a surface dressing. Any surface dressing may be used but usually I prefer to use a cellulose compound or a boiled oil dressing, such as usually is employed in coating split leather, or a surface dressing of rubber is desirable for many uses. This step contemplates all usual methods employed in coating leather by hand, or by use of a knife as is employed in making artificial leather, or when a rubber surface dressing is desired it may be coated under a knife or by impressing a thin coating of rubber compound on the surface on a calendar coating roll. If the web of textile fabric is not employed for supporting the bat or sheet during the coating operation, both sides of the bat or sheet may simultaneously be coated with a suitable surface dressing.
- Many methods are employed in coating leather or woven fabric, any one of which may be employed to secure a similar result in this product and I do not limit myself to any one method for coating nor to any surface dressing. In employing a cellulose, I prefer to press or rub in the first coat of the dressing by passing the sheet between pressure rolls to press the coating into the fibrous surface, or pass the sheet under a knife and then to a friction roller where the coating element is frictioned into the fibrous surface, after which the succeeding coats of the dressing are applied under a knife. In applying an oil dressing I prefer to first coat the fibrous sheet with several coats of cellulose compound and finish the product with the oil dressing imposed on the cellulose dressing.
- When the dressing is desired to be composed of rubber, several coats of rubber compound in liquid form may be imposed on the sheet under a knife, or one or more coats may be placed on the sheet by the knife coating method, and a finishing coat may be impressed to the rubber coated surface between calendar rolls. This product may be of any desired color and may be printed in one or more colors as rubber sheeting is printed, or it may be embossed in any design desired, after which the surface coating of rubber is vulcanized. When rubber is used for the surface dressing I prefer to use a rubber compound as my adhesive agent.
- The next step is to strip the surface dressing and a part of the fibrous material in which it is embedded from the woven fabric, or if the woven fabric is not used then to split or cleave the fibrous sheet. It will be found that the surface coating can be readily split from the laminated sheet, or the fiber sheet when coated on both sides is easily split by starting the sheet to split by hand, and then attaching the ends to wooden shells or paper cores which revolve in oppo-

site directions to pull the sheet apart. The split thus produced will be found to be composed of the surface dressing embedded in a thin untwisted fiber sheet, having considerable strength above the natural strength of the coating film alone and it may be pasted to any surface as for book binding, wall covering, panels, etc. It can be embossed in any design desired either before attaching to another surface or when a fibrous board is used it may be embossed after it is cemented to the board and will in any case retain the embossed design in the same manner that embossed leather buffering retains its embossing.

In the accompanying drawings the steps constituting the above process are illustrated diagrammatically. The numeral 1 indicates a roll of the sheet or bat of unspun fibers. This bat as previously stated consists of superposed strata B', B<sup>2</sup> as indicated in Fig. 2 having a distinct plane of cleavage b between its outer surfaces. This bat is brought into contact with the upper run 2 of an endless conveyor belt and a suitable liquid impregnating medium is fed from a hopper 3 onto the upper surface of the bat. The bat travels with the conveyor between pressure rolls 4 where the impregnating medium is worked thoroughly into the substance of the bat, the product of this operation being indicated in Fig. 3. The bat with its impregnating solution then passes into a drying chamber 5 preferably between pairs of tension rolls 7 and 8 which may be of different diameters so that the bat is subjected to tension during the drying process. Suitable heating coils 6 are arranged within the drying chamber and if the impregnating solution be of rubber, the temperature in the drying chamber may be such as to vulcanize the rubber solution. From the drying chamber the dried bat passes beneath a hopper 9 from which adhesive solution is fed on to the upper surface of the bat. The bat then passes over a guide roller 10 and moves in substantially parallel relation to a web W of textile fabric. This web may conveniently be supplied from a roll 11 and is moved in a horizontal run 12 where adhesive solution is distributed over its upper surface from the hopper 13. The web then passes downwardly as at 14 parallel to the run 15 of the bat, and the two are then brought into contact in passing beneath a roller 16 the adhesive material forming a thin layer C uniting the bat and web. The composite sheet now passes between pressure rolls 17 and 18 which squeeze the bat and web into intimate contact and the composite sheet then passes into a drying or vulcanizing chamber 19 having a heating coil 20. In passing through this chamber, the textile web is beneath the fibrous bat and on emerging from the chamber a suitable surface coating is

applied to the upper face of the bat by means of a hopper 21 and a spreading knife 22. If desired the composite sheet then passes beneath pressure rolls 23 and may 5 then receive a further surface coating or dressing from the hopper 24 and distributing means 25. If desired a further coat of 10 surface dressing may be applied by calendar rolls 27 one of which is furnished with a film of dressing from a hopper 26. The composite sheet after thorough drying now 15 passes about the roller 28 and between splitting rolls 29 and 30 from which point the textile web W diverges from the layer of surface dressing indicated at S.

As the layer of surface dressing is pulled away from the web it carries with it one of the original layers or strata of the bat so that the layer of surface dressing has a 20 stratum of unspun fibers adhering to and embodied in one of its surfaces. The web W having the remainder of the original bat adhering to it may be wound up upon the roller 31 while the split or sheet of artificial buffering 25 S comprising the layer of surface dressing with adhering loose fibers is preferably passed between embossing rolls 32 which impress the layer of surface dressing in such manner as to simulate leather. From these 30 rolls the sheet of artificial leather passes to a roller 33 where it is wound up.

It is obvious that if any of the suggested variations of the process are to be practiced the apparatus for carrying it into effect as 35 above described will be suitably modified.

Having described my invention, what I desire to secure by Letters Patent and claim is:

1. That process of making buffering leather 40 which comprises forming a bat consisting of a plurality of separable layers of unspun fibers, impregnating the bat with adhesive, drying and pressing the bat under tension, coating one side of the bat with a rubber 45 solution, vulcanizing the coating of rubber, and splitting the coated side of the bat from the other side to leave the vulcanized rubber coating with a very thin layer of fibers adhering to one side of it.

2. That process of making buffering leather which comprises forming a bat consisting of a plurality of layers of unspun fibers, impregnating the bat with adhesive, treating the bat to cause the adhesive to set, applying 55 a surface dressing to one side of the bat, treating the bat to cause said dressing to set, and splitting the bat to separate the dressed side from the other side, thereby leaving the split side fibrous and rough.

3. That process of making buffering leather 60 which comprises making a bat of unspun fibers having a cleavage plane intermediate its outer surfaces, impregnating the bat with adhesive, drying the bat, pressing it while under tension to remove wrinkles, applying

a surface dressing to one side of the bat, causing said dressing to solidify, splitting the dressed side of the bat from the other side to leave the solidified dressing with a thin layer of fibers adhering to its surface, 70 and embossing said dressing with its layer of adhering fibers.

4. That process of making buffering leather which comprises making a bat of unspun fibers having a cleavage plane intermediate 75 its outer surfaces impregnating the bat with adhesive, drying the bat, coating one side of the dried bat with adhesive, pressing the coated side of the bat into contact with a textile web, coating the opposite side of the bat with a surface dressing, permitting the dressing to set, and separating that side of the bat which adheres to the web from the dressed side to leave a sheet of solidified dressing with a very thin fibrous layer 80 adhering to its surface.

5. That process of making buffering leather which comprises forming a bat consisting of a plurality of separable layers of unspun fibers, impregnating the bat with adhesive, 90 drying it, coating one side of the bat with rubber solution, coating one side of a textile web with rubber solution, bringing the coated surfaces of the bat and web into contact, pressing the composite sheet, vulcanizing the composite sheet, coating the exposed face of the bat with a surface dressing, causing the dressing to solidify, and splitting off the layer of solidified dressing with a thin stratum of adhering fibers from 95 the composite sheet.

6. That process of making buffering leather which comprises forming a bat consisting of 100 separable strata of unspun fibers, impregnating the bat with adhesive, drying the bat, 105 uniting a textile web to one surface of the bat to form a composite sheet, coating the opposite surface of the bat with a surface dressing consisting of a solution of rubber, vulcanizing the sheet to solidify the rubber, 110 and splitting the rubber coated side of the sheet from the remainder to form a layer of vulcanized rubber having a thin stratum of fibers adhering to one side thereof.

7. The herein described process of making 115 sheet material which comprises preparing a non-woven fibrous bat by impregnating the same with a flexible binding compound, and splitting the impregnated fibrous non-woven material to produce a sheet having a roughened binding face.

8. The herein described process of making 120 artificial leather splits comprising preparing a bat of unwoven unspun fibres, impregnating said bat with an elastic binding agent 125 whereby to coat the individual fibres thereof and consolidate them, splitting the impregnated bat so that the separation of the coated fibres adjacent to the plane of separation between the separating splits will produce a 130

roughened binding surface, and finishing one face of a split so prepared to resemble leather.

9. The herein described process of making sheet material which comprises forming a base material of superposed layers of non-woven fibrous material, impregnating with a flexible binding compound, and separating said base material to form sheets each having a roughened binding surface formed by the separation of the contiguous impregnated fibrous layers.

10. The herein described process of making sheet material which consists in preparing a bat of non-woven felted material, impregnating said bat under pressure with a flexible plastic binding compound whereby to coat the fibres and consolidate them, dividing the impregnated and consolidated bat to form splits each having a roughened binding surface, and finishing one surface of one at least of said splits.

11. Sheet material comprising a bat of unspun and unwoven fibres impregnated with a flexible binding agent, one face of said bat being rough and fibrous and adapted readily to absorb adhesive.

12. Sheet material comprising a bat of unspun and unwoven fibres impregnated and consolidated by means of a flexible binding agent, the ends of certain of the fibres projecting from the plane of one face of the bat whereby said face is rendered rough.

13. Sheet material comprising a layer of unspun unwoven fibres impregnated with an elastic binding agent, said layer having a stratum of solidified surface dressing adhering directly to one of its faces, the opposite face of the layer being fibrous and rough.

14. A fabric comprising a bat of unspun, unwoven fibers impregnated with vulcanized rubber, and a layer of flexible material covering one face of the bat, the other face of the bat being rough and villous.

15. Artificial buffing leather consisting solely of a sheet of solidified dressing having a thin stratum of unspun fibers adhering to one side only thereof, said stratum of fibers being impregnated with a binding adhesive agent and having loose ends of fibers projecting from its outer surface.

16. Artificial buffing leather consisting solely of a thin sheet of vulcanized rubber having a thin layer of unspun cotton fibers adhering to and embedded in one side thereof, said fibrous layer being impregnated with a binding adhesive agent and having loose projecting ends of fibers making its outer surface rough.

Signed at the borough of Manhattan, city of New York, in the county of New York and State of New York, this 28th day of May, A. D. 1920.

ROLAND B. RESPRESS.